# EUROPEAN PATENT SPECIFICATION

(11) **EP 4 016 559 B1**
(45) Date of publication and mention of the grant of the patent: **13.03.2024**
(21) Application number: 20889698.5
(22) Date of filing: 07.07.2020
(51) Int. Cl.: H01F 1/057, H01F 41/02, B22F 9/02, B22F 9/04, C22C 28/00, C22C 30/00, C22C 33/04, C22C 38/00, C22C 38/02, C22C 38/04, C22C 38/10, C22C 38/12, C22C 38/14, C22C 38/16

(54) **NEODYMIUM-IRON-BORON MAGNET MATERIAL, RAW MATERIAL COMPOSITION, PREPARATION METHOD THEREFOR AND USE THEREOF**
NEODYM-EISEN-BOR-MAGNETMATERIAL, ROHSTOFFZUSAMMENSETZUNG, VERFAHREN ZU IHRER HERSTELLUNG UND IHRE VERWENDUNG
MATÉRIAU MAGNÉTIQUE EN NÉODYME-FER-BORE, COMPOSITION DE MATIÈRES PREMIÈRES, SON PROCÉDÉ DE PRÉPARATION ET UTILISATION ASSOCIÉE

(30) Priority: 21.11.2019 CN 201911150996
(43) Date of publication of application: 22.06.2022
(73) Proprietor: Fujian Golden Dragon Rare-Earth Co., Ltd., Longyan City, Fujian Province 366300 (CN)
(72) Inventor: FU, Gang, Longyan, Fujian 366300 (CN); HUANG, Jiaying, Xiamen, Fujian 361000 (CN); HUANG, Jixiang, Longyan, Fujian 366300 (CN); QUAN, Qichen, Longyan, Fujian 366300 (CN)
(74) Representative: karo IP
(86) International application number: PCT/CN2020/100586
(87) International publication number: WO 2021/098223

(56) References cited:
- CN-A- 103 077 796
- CN-A- 103 366 918
- CN-A- 104 064 346
- CN-A- 105 513 737
- CN-A- 106 128 673
- CN-A- 108 730 086
- CN-A- 110 957 091
- JP-A- H08 264 308
- JP-A- 2013 225 533
- JP-A- 2018 056 334
- JP-A- 2019 169 542
- US-A1- 2010 003 156

## Description

### Technical Field

The present disclosure relates to neodymium-iron-boron magnet material and raw material composition, preparation method therefor and use thereof.

### Background

The neodymium-iron-boron (NdFeB) magnet material with Nd₂Fe₁₄B as the main component has high remanence (referred to as Br), coercive force and maximum energy product (referred to as BHmax), which has excellent comprehensive magnetic properties, and can be used in wind power generation, new energy vehicles, inverter appliances, etc. At present, the rare earth component in the neodymium-iron-boron magnet materials in the prior art is usually mainly neodymium, with only a small amount of praseodymium. At present, although there are a few reports in the prior art that replacing a part of neodymium with praseodymium can improve the performance of the magnet material, the degree of improvement is limited, there is still no significant improvement, and relatively expensive heavy rare earth elements need to be added.

### Content of the present invention

The technical problem to be solved in the present disclosure is for overcoming the defect that the coercive force and remanence of the magnet material cannot be significantly improved after replacing the neodymium with praseodymium partially in the prior art, and the present disclosure provides neodymium-iron-boron magnet material, raw material composition, preparation method therefor and use thereof. The neodymium-iron-boron magnet material in the present disclosure increases the content of praseodymium and gallium at the same time, which can overcome the defect in the prior art that the coercivity cannot be significantly improved by increasing the high praseodymium or the high gallium alone, and the remanence and coercive force of the resulting neodymium-iron-boron magnet material are both relatively high without adding a heavy rare earth element.

The present disclosure solves the above technical problems through the following technical solutions.

The present invention provides a raw material composition of neodymium-iron-boron magnet material according to claim 1, dependent claims 2-4 further limit the composition.

The present invention further provides a preparation method for neodymium-iron-boron magnet material, which employs the above-mentioned raw material composition of neodymium-iron-boron magnet material for preparing, according to claim 5.

In the present disclosure, the preparation method comprises the following steps: the molten liquid of the raw material composition of neodymium-iron-boron magnet material is subjected to melting and casting, hydrogen decrepitation, forming, sintering and ageing treatment.

In the present disclosure, the molten liquid of the raw material composition of neodymium-iron-boron magnet material can be prepared by conventional methods in the art, for example, by melting in a high-frequency vacuum induction melting furnace. The vacuum degree of the melting furnace can be 5×10⁻²Pa. The temperature of the melting can be 1500°C or less.

In the present disclosure, the process of the casting can be a conventional casting process in the art, for example: cooling in an Ar gas atmosphere (e.g. in an Ar gas atmosphere of 5.5×10⁴ Pa) at a rate of 10² °C/sec-10⁴ °C/sec.

In the present disclosure, the process of the hydrogen decrepitation can be a conventional hydrogen decrepitation process in the art. For example, being subjected to hydrogen absorption, dehydrogenation and cooling treatment.

Wherein, the hydrogen absorption can be carried out under the condition of a hydrogen pressure of 0.15 MPa.

Wherein, the dehydrogenation can be carried out under the condition of heating up while vacuum-pumping.

In the present disclosure, the process of the pulverization after hydrogen decrepitation can be a conventional pulverization process in the art, for example jet mill pulverization. The jet mill pulverization can be preferably carried out under a nitrogen atmosphere with an oxidizing gas content of 150 ppm or less. The oxidizing gas refers to the content of oxygen or moisture. The pressure in the pulverizing chamber of the jet mill pulverization can be preferably 0.38 MPa; the time for the jet mill pulverization can be preferably 3 hours.

Wherein, after the pulverization, a lubricant, for example zinc stearate, can be added to powder according to conventional means in the art. The addition amount of the lubricant can be 0.10-0.15%, for example 0.12%, by weight of the mixed powder.

In the present disclosure, the process of the forming can be a conventional forming process in the art, for example a magnetic field forming method or a hot pressing and hot deformation method.

In the present disclosure, the process of sintering can be a conventional sintering process in the art. For example, preheating, sintering and cooling under vacuum conditions (e.g. under a vacuum of 5×10⁻³ Pa).

Wherein, the temperature of preheating can be 300-600°C. The time of preheating can be 1-2 h. Preferably, the preheating is performed for 1 h at a temperature of 300°C and 600°C, respectively.

Wherein, the temperature of sintering is preferably 1030-1080°C, for example 1040°C.

Wherein, the time of sintering can be a conventional sintering time in the art, for example 2h.

Wherein, the cooling can be preceded by passing Ar gas to bring the air pressure to 0.1 MPa.

In the present disclosure, after sintering and before the ageing treatment, a grain boundary diffusion treatment is preferably further carried out.

Wherein, the grain boundary diffusion treatment can be carried out by a conventional process in the art. For example, substance containing Tb and/or substance containing Dy is attached to the surface of the neodymium-iron-boron magnet material by evaporating, coating or sputtering, and then diffusion heat treatment is carried out.

The substance containing Tb can be a Tb metal, a Tb-containing compound, for example a Tb-containing fluoride or an alloy.

The substance containing Dy can be a Dy metal, a Dy-containing compound, for example a Dy-containing fluoride or an alloy.

The temperature of the diffusion heat treatment can be 800-900°C, for example 850°C.

The time of the diffusion heat treatment can be 12-48h, for example 24h.

In the present disclosure, in the ageing treatment, the temperature of the secondary ageing treatment is preferably 460-650°C, for example 500°C.

In the present disclosure, in the secondary ageing treatment, the temperature is increased to 460-650°C preferably at a heating rate of 3-5°C/min. The starting point of the temperature increase can be room temperature.

The present invention provides a neodymium-iron-boron magnet material according to claim 6, produced from the raw material composition of claims 1-4. Dependent claims 7 and 8 further limit the magnet material composition. Claim 9 specifies the use in a motor.

The reagents and raw materials used in the present disclosure are commercially available.

The positive progress of the present invention is as follows: in the prior art, adding praseodymium and gallium to the neodymium-iron-boron magnet material can increase the coercivity, but reduce the remanence at the same time. The inventor provided a large number of experiments and found that the compatibility of specific content of praseodymium and gallium can produce a synergistic effect, that is, adding specific content of praseodymium and gallium at the same time can significantly improve the coercivity of neodymium-iron-boron magnet material, and only slightly reduce the remanence. And the remanence and coercive force of the magnet material in the present disclosure are both relatively high without adding a heavy rare earth element.

### Brief description of the drawings

Figure1 shows the element distribution diagram formed by FE-EPMA surface scan of the neodymium-iron-boron magnet material prepared in Example 23.
Figure 2 shows the element distribution diagram at the grain boundary of the neodymium-iron-boron magnet material prepared in Example 23, and 1 in the figure shows the point taken by quantitative analysis at the grain boundary.
Figure 3 shows the element distribution diagram of the intergranular triangular region of the neodymium-iron-boron magnet material prepared in Example 23, and 1 in the figure shows the point taken by quantitative analysis in the intergranular triangular region.

### Detailed description of the preferred embodiment

The following examples further illustrate the present disclosure, but the present disclosure is not limited thereto. Experiment methods in which specific conditions are not indicated in the following embodiments are selected according to conventional methods and conditions, or according to the product specification. The wt.% in the following tables refers to the mass percentage of the content of each component in the total mass of the raw material composition of neodymium-iron-boron magnet material, and "/" indicates that the element was not added. "Br" refers to the residual magnetic flux density and "Hcj" refers to the intrinsic coercivity.

The formulations of the raw material compositions of the neodymium-iron-boron magnet material in the examples and the comparative examples are shown in Table 1 below.

Table 1 Formulations for the raw material compositions of the neodymium-iron-boron magnet materials in the examples and the comparative examples (wt.%)

| No. | Nd | Pr | Dy | Tb | Ho | Ga | Cu | A1 | Zr | Co | Mn | Zn | Mo | B | Fe |
|---|---|---|---|---|---|---|---|---|---|---|---|---|---|---|---|
| 1 | 13.85 | 17.15 | / | / | / | 0.25 | / | / | / | / | / | / | / | 0.985 | 67.765 |
| 2 | 13.85 | 17.15 | / | / | / | 0.27 | / | / | / | / | / | / | / | 0.985 | 67.745 |
| 3 | 12.35 | 18.15 | / | / | / | 0.29 | / | / | / | / | / | / | / | 0.985 | 68.225 |
| 4 | 12.85 | 18.15 | / | / | / | 0.31 | / | / | / | / | / | / | / | 0.985 | 67.705 |
| 5 | 12.35 | 19.15 | / | / | / | 0.33 | / | / | / | / | / | / | / | 0.985 | 67.185 |
| 6 | 12.85 | 19.15 | / | / | / | 0.35 | / | / | / | / | / | / | / | 0.985 | 66.665 |
| 7 | 11.35 | 20.15 | / | / | / | 0.37 | / | / | / | / | / | / | / | 0.985 | 67.145 |
| 8 | 11.35 | 20.15 | / | / | / | 0.39 | / | / | / | / | / | / | / | 0.985 | 67.125 |
| 9 | 10.85 | 21.15 | / | / | / | 0.41 | / | / | / | / | / | / | / | 0.985 | 66.605 |
| 10 | 10.65 | 21.15 | / | / | / | 0.43 | / | / | / | / | / | / | / | 0.985 | 66.785 |
| 11 | 8.85 | 22.15 | / | / | / | 0.45 | / | / | / | / | / | / | / | 0.95 | 67.6 |
| 12 | 7.85 | 23.15 | / | / | / | 0.47 | / | / | / | / | / | / | / | 0.96 | 67.57 |
| 13 | 6.85 | 24.15 | / | / | / | 0.49 | / | / | / | / | / | / | / | 0.97 | 67.54 |
| 14 | 5.85 | 25.15 | / | / | / | 0.6 | / | / | / | / | / | / | / | 0.98 | 67.42 |
| 15 | 4.85 | 26.15 | / | / | / | 0.7 | / | / | / | / | / | / | / | 0.99 | 67.31 |
| 16 | 3.85 | 27.15 | / | / | / | 0.8 | / | / | / | / | / | / | / | 0.985 | 67.215 |
| 17 | 2.85 | 27.85 | / | / | / | 0.9 | / | / | / | / | / | / | / | 0.985 | 67.415 |
| 18 | 1.85 | 28.85 | / | / | / | 1.0 | / | / | / | / | / | / | / | 0.985 | 67.315 |
| 19 | 13.65 | 17.15 | / | / | / | 0.3 | 0.1 | / | / | / | / | / | / | 0.985 | 67.815 |
| 20 | 13.35 | 17.15 | / | / | / | 0.47 | 0.25 | / | / | / | / | / | / | 0.985 | 67.795 |
| 21 | 10.85 | 21.15 | / | / | / | 0.53 | 0.5 | / | / | / | / | / | / | 0.985 | 65.985 |
| 22 | 10.85 | 21.15 | / | / | / | 1.0 | 0.7 | / | / | / | / | / | / | 0.985 | 65.315 |
| 23 | 7.85 | 23.15 | / | / | / | 0.49 | / | 0.2 | / | / | / | / | / | 0.985 | 67.325 |
| 24 | 7.85 | 23.15 | / | / | / | 0.51 | / | 0.45 | / | / | / | / | / | 0.985 | 67.055 |
| 25 | 5.85 | 24.15 | / | 2 | / | 0.53 | / | 0.6 | / | / | / | / | / | 1 | 65.87 |
| 26 | 5.85 | 24.15 | 0.3 | 1.7 | / | 0.55 | / | 0.8 | / | / | / | / | / | 1.1 | 65.55 |
| 27 | 9.85 | 20.15 | 0.3 | 1.2 | / | 0.57 | / | / | 0.1 | / | 0.01 | / | / | 1.2 | 66.62 |
| 28 | 9.85 | 20.15 | 0.1 | 1.4 | / | 0.28 | / | / | 0.25 | / | 0.015 | / | / | 1.2 | 66.755 |
| 29 | 11.15 | 20.15 | / | 0.5 | / | 0.32 | / | / | 0.28 | / | 0.013 | / | / | 0.985 | 66.602 |
| 30 | 11.15 | 20.15 | / | 0.5 | / | 0.36 | / | / | 0.3 | / | 0.018 | / | / | 0.985 | 66.537 |
| 31 | 6.15 | 23.15 | 0.1 | 1.5 | / | 0.7 | / | / | 0.35 | / | / | / | / | 0.985 | 67.065 |
| 32 | 6.15 | 23.15 | 0.2 | 1.4 | / | 0.8 | / | / | 0.4 | / | / | / | / | 0.985 | 66.915 |
| 32.1 | 7.85 | 23.15 | 0.5 | / | / | 0.85 | / | / | 0.25 | / | 0.01 | / | / | 0.985 | 66.405 |
| 32.2 | 7.85 | 23.15 | / | 1 | / | 0.95 | / | / | 0.3 | / | 0.013 | / | / | 0.985 | 65.752 |
| 33 | 6.85 | 24.15 | 0.3 | 0.7 | / | 1.0 | / | / | / | 1 | / | / | / | 0.985 | 65.015 |
| 34 | 6.85 | 24.15 | 0.3 | 0.7 | / | 0.25 | 0.1 | 0.2 | / | / | / | / | / | 0.985 | 66.465 |
| 35 | 6.85 | 24.15 | 0.3 | 0.7 | / | 0.4 | 0.2 | 0.4 | / | / | / | / | / | 0.985 | 66.015 |
| 36 | 5.85 | 24.15 | 0.2 | 0.8 | / | 0.5 | 0.4 | 0.6 | / | / | / | / | / | 0.985 | 66.515 |
| 37 | 5.85 | 24.15 | 0.2 | 0.8 | / | 1.0 | 0.8 | 1 | / | / | / | / | / | 0.985 | 65.215 |
| 38 | 12.35 | 19.15 | / | / | / | 0.3 | 0.2 | / | 0.1 | / | / | / | / | 0.985 | 66.915 |
| 39 | 11.75 | 19.15 | / | / | / | 1.0 | 0.4 | / | 0.25 | / | / | / | / | 0.985 | 66.465 |
| 40 | 12.35 | 17.15 | 0.3 | 0.7 | / | 0.3 | / | 0.05 | 0.1 | / | / | / | / | 0.985 | 68.065 |
| 41 | 12.35 | 17.15 | 0.3 | 0.7 | / | 0.35 | / | 0.1 | 0.25 | / | / | / | / | 0.985 | 67.815 |
| 42 | 11.75 | 19.15 | / | / | / | 0.45 | / | 0.3 | 0.28 | / | / | / | / | 0.985 | 67.085 |
| 43 | 11.75 | 19.15 | / | / | / | 0.6 | / | 0.6 | 0.3 | / | / | / | / | 0.985 | 66.615 |
| 44 | 12.85 | 18.15 | / | / | / | 0.25 | 0.35 | 0.02 | 0.15 | / | / | / | / | 0.985 | 67.245 |
| 45 | 12.85 | 18.15 | / | / | / | 0.28 | 0.45 | 0.03 | 0.25 | / | / | / | / | 0.985 | 67.005 |
| 46 | 11.75 | 19.15 | / | / | / | 0.36 | 0.48 | 0.1 | 0.26 | / | / | / | / | 0.985 | 66.915 |
| 47 | 11.75 | 19.15 | / | / | / | 0.38 | 0.5 | 0.03 | 0.27 | / | / | / | / | 0.985 | 66.935 |
| 48 | 9.85 | 20.15 | 0.2 | 1 | / | 0.55 | 0.55 | 0.02 | 0.28 | / | / | / | / | 0.985 | 66.415 |
| 49 | 9.85 | 20.15 | 0.2 | 1 | / | 0.6 | 0.58 | 0.03 | 0.29 | / | / | / | / | 0.985 | 66.315 |
| 49.1 | 6.15 | 23.15 | / | 2 | / | 0.7 | 0.35 | 0.02 | 0.25 | / | / | / | / | 0.985 | 66.395 |
| 49.2 | 6.15 | 23.15 | / | 1 | / | 0.8 | 0.45 | 0.02 | 0.25 | / | / | / | / | 0.985 | 67.195 |
| 49.3 | 5.85 | 25.15 | 1 | | / | 0.9 | 0.45 | 0.03 | 0.3 | / | / | / | / | 0.985 | 65.335 |
| 49.4 | 5.85 | 25.15 | / | / | / | 1 | 0.5 | 0.03 | 0.3 | / | / | / | / | 0.985 | 66.185 |
| 50 | 9.55 | 20.15 | 0.2 | 1 | 1 | 0.3 | / | 0.05 | / | / | / | 0.02 | 0.05 | 0.985 | 66.695 |
| 51 | 11.75 | 19.15 | / | / | 1 | 0.45 | / | 0.12 | / | / | / | 0.05 | 0.02 | 0.985 | 66.475 |
| 52 | 12.85 | 18.15 | / | / | 1 | 0.6 | / | 0.15 | / | / | / | 0.05 | 0.05 | 0.985 | 66.165 |
| 55 | 6.85 | 24.15 | / | / | / | 0.1 | 0.1 | 0.2 | / | / | / | / | / | 0.985 | 67.615 |
| 56 | 6.85 | 24.15 | / | / | / | 0.2 | 0.1 | 0.2 | / | / | / | / | / | 0.985 | 67.515 |
| 57 | 15.15 | 15.85 | / | / | / | 0.25 | 0.1 | 0.2 | / | / | / | / | / | 0.985 | 67.465 |
| 58 | 22.15 | 8.85 | / | / | / | 0.25 | 0.1 | 0.2 | / | / | / | / | / | 0.985 | 67.465 |

### Example 1

The neodymium-iron-boron magnet materials were prepared as follows:
(1) Melting and casting process: according to the formulations shown in Table 1, the prepared raw materials were put into a crucible made of alumina and vacuum melted in a high-frequency vacuum induction melting furnace and in a vacuum of 5 × 10⁻² Pa at a temperature of 1500°C or less. After vacuum melting, the melting furnace was fed with Ar gas to make the air pressure reach 5.5 × 10⁴ Pa and then casting was carried out, and a cooling rate of 10²°C/sec - 10⁴°C/sec was used to obtain the quench alloy.
(2) Hydrogen decrepitation process: the melting furnace with quench alloy placed therein was evacuated at room temperature, and then hydrogen gas of 99.9% purity was passed into the furnace for hydrogen decrepitation to maintain the hydrogen pressure at 0.15 MPa; after sufficient hydrogen absorption, it was sufficiently dehydrogenated by heating up while vacuum-pumping; then it was cooled and the powder after hydrogen decrepitation was taken out.
(3) Micro-pulverization process: the powder after hydrogen decrepitation was pulverized by jet mill for 3 hours in nitrogen atmosphere with oxidizing gas content of 150 ppm or less and under the condition of the pressure of 0.38 MPa in the pulverization chamber, and fine powder was obtained. The oxidizing gas refers to oxygen or moisture.
(4) Zinc stearate was added to the powder after jet mill pulverization, and the addition amount of zinc stearate was 0.12% by weight of the mixed powder, and then it was mixed thoroughly by using a V-mixer.
(5) Magnetic field forming process: a rectangular oriented magnetic field forming machine was used to conduct primary forming of the above-mentioned powder with zinc stearate into a cube with sides of 25 mm in an orientation magnetic field of 1.6 T and a forming pressure of 0.35 ton/cm²; after the primary forming, it was demagnetized in a magnetic field of 0.2 T. In order to prevent the formed body after the primary forming from contacting with air, it was sealed, and then secondary forming was carried out at a pressure of 1.3 ton/cm² using a secondary forming machine (isostatic forming machine).
(6) Sintering process: each formed body was moved to a sintering furnace for sintering, the sintering was maintained under a vacuum of 5×10⁻³ Pa and at a temperature of 300 °C and 600 °C for 1 hour, respectively; then, sintered at a temperature of 1040°C for 2 hours; and then Ar gas was passed in to make the air pressure reach 0.1 MPa, and cooled to room temperature to obtain sintered body.
(7) Ageing treatment process: the sintered body was heat treated in high purity Ar gas at a temperature of 500°C for 3 hours and then cooled to room temperature and taken out.

### Example 53 Using Dy grain boundary diffusion method

The raw material composition of Example 1 in Table 1 was first prepared according to the preparation of the sintered body of Example 1 to obtain a sintered body, followed by grain boundary diffusion, and then aging treatment. Wherein the process of aging treatment is the same as in Example 1, and the processing procedure of grain boundary diffusion is as follows:

The sintered body was processed into a magnet with a diameter of 20 mm and a thickness of less than 3 mm, and the thickness direction is the magnetic field orientation direction, after the surface was cleaned, the raw materials formulated with Dy fluoride were used to coat the magnet through a full spray, and the coated magnet was dried, and the metal with Tb element was attached to the magnet surface by sputtering in a high-purity Ar gas atmosphere, diffusion heat treatment was carried out at a temperature of 850°C for 24 hours. Cooled to room temperature.

### Example 54 Using Tb grain boundary diffusion method

The number 1 in Table 1 was first prepared according to the preparation of the sintered body of Example 1 to obtain a sintered body, followed by grain boundary diffusion, and then aging treatment. Wherein the process of aging treatment is the same as in Example 1, and the processing procedure of grain boundary diffusion is as follows:

The sintered body was processed into a magnet with a diameter of 20 mm and a thickness of less than 7 mm, and the thickness direction is the magnetic field orientation direction, after the surface was cleaned, the raw materials formulated with Tb fluoride were used to coat the magnet through a full spray, and the coated magnet was dried, and the metal with Tb element was attached to the magnet surface by sputtering in a high-purity Ar gas atmosphere, diffusion heat treatment was carried out at a temperature of 850°C for 24 hours. Cooled to room temperature.

### Effect Example

The magnetic properties and compositions of the neodymium-iron-boron magnet materials made in Examples 1-54 and Comparative Examples 55-58 were measured, and the crystalline phase structure of the magnets was observed using a field emission electron probe microanalyzer (FE-EPMA).
(1) Magnetic properties evaluation: The magnetic properties were examined using the NIM-10000H type BH bulk rare earth permanent magnet nondestructive measurement system in National Institute of Metrology, China. The following Table 2 indicates the magnetic property testing results, wherein 1kG=0.1T and 1kOe=79.6kA/m.

**Table 2**

| No. | Br(kGs) | Hcj(kOe) | Absolute value of Hcj temperature coefficient at 80°C | Absolute value of Hcj temperature coefficient at 150°C | Absolute value of Hcj temperature coefficient at 180°C |
|---|---|---|---|---|---|
| 1 | 14.12 | 18.24 | 0.689 | / | / |
| 2 | 14.09 | 18.38 | 0.685 | / | / |
| 3 | 14.34 | 18.07 | 0.692 | / | / |
| 4 | 14.21 | 18.55 | 0.672 | / | / |
| 5 | 13.90 | 19.52 | 0.668 | / | / |
| 6 | 13.79 | 19.88 | 0.664 | / | / |
| 7 | 13.81 | 20.04 | 0.648 | / | / |
| 8 | 13.79 | 20.18 | 0.642 | / | / |
| 9 | 13.72 | 20.79 | 0.638 | / | / |
| 10 | 13.74 | 20.84 | 0.632 | / | / |
| 11 | 13.91 | 20.88 | 0.631 | / | / |
| 12 | 13.93 | 21.27 | 0.612 | / | / |
| 13 | 13.88 | 21.52 | 0.609 | / | / |
| 14 | 13.73 | 22.66 | 0.591 | / | / |
| 15 | 13.58 | 23.55 | 0.577 | / | / |
| 16 | 13.46 | 24.52 | / | 0.532 | |
| 17 | 13.38 | 25.01 | / | 0.518 | / |
| 18 | 13.23 | 25.8 | / | 0.513 | / |
| 19 | 14.07 | 19.03 | 0.673 | / | / |
| 20 | 13.92 | 20.18 | 0.649 | / | / |
| 21 | 13.05 | 24.07 | / | 0.556 | / |
| 22 | 12.45 | 28.23 | / | 0.503 | / |
| 23 | 13.98 | 21.88 | 0.623 | / | / |
| 24 | 13.75 | 22.61 | 0.617 | / | / |
| 25 | 12.7 | 30.6 | / | / | 0.437 |
| 26 | 12.5 | 30.9 | / | / | 0.435 |
| 27 | 13.35 | 26.2 | / | 0.513 | / |
| 28 | 13.4 | 24.64 | / | 0.530 | / |
| 29 | 13.6 | 21.75 | 0.605 | / | / |
| 30 | 13.57 | 22.03 | 0.619 | / | / |
| 31 | 13.82 | 26.32 | / | 0.509 | / |
| 32 | 13.75 | 26.91 | / | 0.506 | / |
| 32.1 | 13.21 | 25.65 | / | 0.518 | |
| 32.2 | 12.79 | 28.89 | / | 0.496 | |
| 33 | 12.7 | 28.63 | / | 0.495 | / |
| 34 | 13.3 | 24.53 | / | 0.535 | / |
| 35 | 13.1 | 26.03 | / | 0.519 | / |
| 36 | 12.95 | 28.33 | / | 0.502 | / |
| 37 | 11.72 | 33.83 | / | / | 0.422 |
| 38 | 13.66 | 20.47 | 0.638 | / | / |
| 39 | 12.9 | 25.9 | / | 0.513 | / |
| 40 | 13.94 | 21.63 | 0.623 | / | / |
| 41 | 13.9 | 22.19 | 0.624 | / | / |
| 42 | 13.93 | 20.97 | 0.633 | / | / |
| 43 | 13.7 | 22.72 | 0.611 | / | / |
| 44 | 13.68 | 20.38 | 0.641 | / | / |
| 45 | 13.47 | 21.17 | 0.629 | / | / |
| 46 | 13.33 | 22.24 | 0.617 | / | / |
| 47 | 13.51 | 22.48 | 0.615 | / | / |
| 48 | 13.09 | 27.27 | / | 0.516 | / |
| 49 | 13.05 | 27.79 | / | 0.512 | / |
| 49.1 | 12.89 | 31.2 | / | / | 0.439 |
| 49.2 | 13.18 | 28.28 | / | 0.492 | / |
| 49.3 | 12.73 | 28.73 | / | 0.488 | / |
| 49.4 | 12.68 | 29.43 | / | 0.471 | / |
| 50 | 13.43 | 23.51 | 0.573 | / | / |
| 51 | 12.85 | 25.57 | / | 0.518 | / |
| 52 | 12.68 | 26.37 | / | 0.512 | / |
| 53 | 13.95 | 24.5 | / | 0.535 | / |
| 54 | 13.98 | 29.3 | / | 0.472 | / |
| 55 | 13.85 | 18.69 | 0.668 | / | / |
| 56 | 13.82 | 18.75 | 0.666 | / | / |
| 57 | 13.95 | 17.51 | 0.672 | / | / |
| 58 | 14.19 | 15.79 | 0.749 | / | / |

(2) Composition determination: the components were determined using a high-frequency inductively coupled plasma emission spectrometer (ICP-OES). The following Table 3 shows the results of the composition testing.

**Table 3 Composition test results (wt.%)**

| No. | Nd | Pr | Dy | Tb | Ho | Ga | Cu | Al | Zr | Co | Mn | Zn | Mo | B | Fe |
|---|---|---|---|---|---|---|---|---|---|---|---|---|---|---|---|
| 1 | 13.848 | 17.151 | / | / | / | 0.248 | / | / | / | / | / | / | / | 0.984 | 67.769 |
| 2 | 13.856 | 17.150 | / | / | / | 0.268 | / | / | / | / | / | / | / | 0.987 | 67.784 |
| 3 | 12.451 | 18.132 | / | / | / | 0.291 | / | / | / | / | / | / | / | 0.983 | 68.143 |
| 4 | 12.89 | 18.148 | / | / | / | 0.312 | / | / | / | / | / | / | / | 0.983 | 67.667 |
| 5 | 12.345 | 19.149 | / | / | / | 0.332 | / | / | / | / | / | / | / | 0.986 | 67.188 |
| 6 | 12.851 | 19.149 | / | / | / | 0.352 | / | / | / | / | / | / | / | 0.984 | 66.664 |
| 7 | 11.355 | 20.147 | / | / | / | 0.371 | / | / | / | / | / | / | / | 0.987 | 67.14 |
| 8 | 11.352 | 20.148 | / | / | / | 0.392 | / | / | / | / | / | / | / | 0.983 | 67.125 |
| 9 | 10.851 | 21.146 | / | / | / | 0.413 | / | / | / | / | / | / | / | 0.983 | 66.607 |
| 10 | 10.651 | 21.148 | / | / | / | 0.433 | / | / | / | / | / | / | / | 0.986 | 66.782 |
| 11 | 8.851 | 22.148 | / | / | / | 0.452 | / | / | / | / | / | / | / | 0.949 | 67.6 |
| 12 | 7.852 | 23.149 | / | / | / | 0.472 | / | / | / | / | / | / | / | 0.956 | 67.571 |
| 13 | 6.853 | 24.151 | / | / | / | 0.492 | / | / | / | / | / | / | / | 0.969 | 67.535 |
| 14 | 5.852 | 25.152 | / | / | / | 0.589 | / | / | / | / | / | / | / | 0.982 | 67.425 |
| 15 | 4.852 | 26.151 | / | / | / | 0.712 | / | / | / | / | / | / | / | 0.991 | 67.294 |
| 16 | 3.848 | 27.152 | / | / | / | 0.82 | / | / | / | / | / | / | / | 0.985 | 67.195 |
| 17 | 2.848 | 27.851 | / | / | / | 0.912 | / | / | / | / | / | / | / | 0.984 | 67.405 |
| 18 | 1.852 | 28.852 | / | / | / | 1.03 | / | / | / | / | / | / | / | 0.987 | 67.279 |
| 19 | 13.651 | 17.149 | / | / | / | 0.301 | 0.1 | / | / | / | / | / | / | 0.983 | 67.816 |
| 20 | 13.348 | 17.147 | / | / | / | 0.471 | 0.25 | / | / | / | / | / | / | 0.983 | 67.801 |
| 21 | 10.848 | 21.148 | / | / | / | 0.531 | 0.5 | / | / | / | / | / | / | 0.984 | 65.989 |
| 22 | 10.849 | 21.148 | / | / | / | 1.02 | 0.7 | / | / | / | / | / | / | 0.987 | 65.296 |
| 23 | 7.849 | 23.148 | / | / | / | 0.491 | / | 0.202 | / | / | / | / | / | 0.983 | 67.327 |
| 24 | 7.849 | 23.147 | / | / | / | 0.512 | / | 0.451 | / | / | / | / | / | 0.983 | 67.058 |
| 25 | 5.848 | 24.148 | / | 2.001 | / | 0.531 | / | 0.603 | / | / | / | / | / | 1.02 | 65.849 |
| 26 | 5.848 | 24.148 | 0.301 | 1.701 | / | 0.551 | / | 0.801 | / | / | / | / | / | 1.11 | 65.54 |
| 27 | 9.848 | 20.148 | 0.302 | 1.21 | / | 0.572 | / | / | 0.1 | / | 0.01 | / | / | 1.19 | 66.62 |
| 28 | 9.848 | 20.149 | 0.101 | 1.42 | / | 0.281 | / | / | 0.25 | / | 0.015 | / | / | 1.18 | 66.756 |
| 29 | 11.149 | 20.154 | / | 0.502 | / | 0.323 | / | / | 0.28 | / | 0.013 | / | / | 0.984 | 66.595 |
| 30 | 11.148 | 20.151 | / | 0.503 | / | 0.361 | / | / | 0.3 | / | 0.018 | / | / | 0.987 | 66.532 |
| 31 | 6.147 | 23.152 | 0.101 | 1.492 | / | 0.703 | / | / | 0.35 | / | / | / | / | 0.983 | 67.072 |
| 32 | 6.148 | 23.152 | 0.202 | 1.402 | / | 0.804 | / | / | 0.4 | / | / | / | / | 0.983 | 66.909 |
| 32.1 | 7.846 | 23.152 | 0.51 | / | / | 0.848 | / | / | 0.248 | / | 0.02 | / | / | 0.984 | 66.392 |
| 32.2 | 7.851 | 23.15 | / | 1.02 | / | 0.951 | / | / | 0.301 | / | 0.014 | / | / | 0.984 | 65.729 |
| 33 | 6.847 | 24.151 | 0.303 | 0.702 | / | 1.03 | / | / | / | 1 | / | / | / | 0.986 | 64.981 |
| 34 | 6.846 | 24.152 | 0.301 | 0.703 | / | 0.252 | 0.102 | 0.202 | / | / | / | / | / | 0.984 | 66.458 |
| 35 | 6.848 | 24.151 | 0.302 | 0.704 | / | 0.402 | 0.205 | 0.402 | / | / | / | / | / | 0.984 | 66.002 |
| 36 | 5.845 | 24.152 | 0.202 | 0.802 | / | 0.502 | 0.405 | 0.602 | / | / | / | / | / | 0.987 | 66.503 |
| 37 | 5.85 | 24.152 | 0.203 | 0.802 | / | 1.03 | 0.803 | 1.02 | / | / | / | / | / | 0.983 | 65.157 |
| 38 | 12.347 | 19.153 | / | / | / | 0.302 | 0.202 | / | 0.1 | / | / | / | / | 0.983 | 66.913 |
| 39 | 11.748 | 19.151 | / | / | / | 1.02 | 0.402 | / | 0.25 | / | / | / | / | 0.984 | 66.445 |
| 40 | 12.347 | 17.149 | 0.301 | 0.703 | / | 0.303 | / | 0.04 | 0.1 | / | / | / | / | 0.987 | 68.07 |
| 41 | 12.35 | 17.145 | 0.301 | 0.705 | / | 0.351 | / | 0.102 | 0.25 | / | / | / | / | 0.983 | 67.813 |
| 42 | 11.746 | 19.146 | / | / | / | 0.451 | / | 0.301 | 0.28 | / | / | / | / | 0.983 | 67.093 |
| 43 | 11.748 | 19.149 | / | / | / | 0.602 | / | 0.601 | 0.3 | / | / | / | / | 0.986 | 66.614 |
| 44 | 12.848 | 18.148 | / | / | / | 0.251 | 0.352 | 0.02 | 0.15 | / | / | / | / | 0.984 | 67.247 |
| 45 | 12.848 | 18.146 | / | / | / | 0.281 | 0.451 | 0.03 | 0.25 | / | / | / | / | 0.987 | 67.007 |
| 46 | 11.751 | 19.149 | / | / | / | 0.362 | 0.481 | 0.101 | 0.26 | / | / | / | / | 0.984 | 66.912 |
| 47 | 11.752 | 19.148 | / | / | / | 0.38 | 0.502 | 0.02 | 0.27 | / | / | / | / | 0.987 | 66.941 |
| 48 | 9.852 | 20.147 | 0.202 | 1.01 | / | 0.55 | 0.552 | 0.02 | 0.28 | / | / | / | / | 0.983 | 66.404 |
| 49 | 9.851 | 20.146 | 0.203 | 1.02 | / | 0.6 | 0.581 | 0.03 | 0.29 | / | / | / | / | 0.983 | 66.296 |
| 49.1 | 6.149 | 23.151 | / | 2.01 | / | 0.701 | 0.351 | 0.01 | 0.251 | / | / | / | / | 0.984 | 66.393 |
| 49.2 | 6.151 | 23.151 | / | 1.02 | / | 0.791 | 0.452 | 0.01 | 0.252 | / | / | / | / | 0.986 | 67.187 |
| 49.3 | 5.852 | 25.152 | 1.03 | / | / | 0.892 | 0.451 | 0.03 | 0.301 | / | / | / | / | 0.984 | 65.308 |
| 49.4 | 5.851 | 25.152 | / | / | / | 1.02 | 0.501 | 0.04 | 0.302 | / | / | / | / | 0.984 | 66.15 |
| 50 | 9.549 | 20.148 | 0.203 | 1.03 | 1.02 | 0.3 | / | 0.05 | / | / | / | 0.01 | 0.06 | 0.986 | 66.644 |
| 51 | 11.747 | 19.148 | / | / | 1.01 | 0.45 | / | 0.12 | / | / | / | 0.06 | 0.03 | 0.984 | 66.451 |
| 52 | 12.848 | 18.146 | / | / | 0.99 | 0.6 | / | 0.15 | / | / | / | 0.04 | 0.03 | 0.987 | 66.209 |
| 53 | 13.849 | 17.152 | 0.421 | / | / | 0.247 | / | / | / | / | / | / | / | 0.984 | 67.347 |
| 54 | 13.848 | 17.151 | / | 0.501 | / | 0.249 | / | / | / | / | / | / | / | 0.984 | 67.267 |
| 55 | 6.846 | 24.148 | / | / | / | 0.1 | 0.101 | 0.2 | / | / | / | / | / | 0.984 | 67.621 |
| 56 | 6.845 | 24.148 | / | / | / | 0.2 | 0.103 | 0.2 | / | / | / | / | / | 0.987 | 67.517 |
| 57 | 15.148 | 15.849 | / | / | / | 0.25 | 0.102 | 0.2 | / | / | / | / | / | 0.983 | 67.468 |
| 58 | 22.146 | 8.849 | / | / | / | 0.25 | 0.102 | 0.2 | / | / | / | / | / | 0.983 | 67.47 |

FE-EPMA inspection: the perpendicularly oriented surface of the magnet material of Example 23 was polished and inspected using a field emission electron probe micro-analyzer (FE-EPMA) (Japan Electronics Corporation (JEOL), 8530F). The main elements analyzed are Pr, Nd, Ga, Zr, O, and the elements at the grain boundary and the intergranular triangular region were quantitatively analyzed.

Figure 1 shows the distribution diagram of each element in the neodymium-iron-boron magnet material. From Figure 1, it can be seen that the Pr and Nd elements are mainly distributed in the main phase, some rare earths also appear in the grain boundary, and the element Ga is also distributed in the main phase and the crystal phase, the element Zr is distributed at the grain boundary.

Figure 2 shows the element distribution at the grain boundary of the neodymium-iron-boron magnet material of Example 23, and the elements at the grain boundary were quantitatively analyzed by taking the point marked by 1 in Figure 2, the results are shown in Table 4 below:

**Table 4**

| Pr (wt.%) | Nd (wt.%) | Ga (wt.%) | Zr (wt.%) | O (wt.%) | Fe (wt.%) |
|---|---|---|---|---|---|
| 37.8 | 28.2 | 5.26 | 0.08 | 0.69 | Bal |

From the above data, it can be clearly seen that Pr and Nd exist in the form of rare earth rich phases and oxides in the grain boundaries, α-Pr and α-Nd, Pr₂O₃, Nd₂O₃ and NdO, respectively, and Ga occupies a certain content of about 5.26wt.% at the grain boundaries in addition to the main phase, Zr is dispersed in the whole region as a high melting point element.

Figure 3 shows the element distribution of the intergranular triangular region of the neodymium-iron-boron magnet materials of Example 23, and the elements in the intergranular triangular region were quantitatively analyzed by taking the point marked by 1 in Figure 3, and the results are shown in Table 5 below:

**Table 5**

| Pr (wt.%) | Nd(wt.%) | Ga (wt.%) | Zr (wt.%) | O (wt.%) | Fe (wt.%) |
|---|---|---|---|---|---|
| 27.8 | 29.5 | 4.95 | 0.039 | 0.95 | Bal |

In the intergranular triangular region, Pr and Nd elements are distributed in it, in the formulations with high Pr, it is clearly found that the content of Pr is obviously lower than that of Nd in the intergranular triangular region, although some rare earths are enriched here, the enrichment degree of Pr is less than that of Nd, which is one of the reasons why high Pr and Ga work together to improve the coercivity. At the same time, there is a partial distribution of O and Ga therein.

## Claims

1. A raw material composition of neodymium-iron-boron magnet material, which comprises the following components by mass percentage, wherein the percentage refers to the mass percentage of the content of each component in the total mass of the raw material composition of neodymium-iron-boron magnet material:
29.5-32% of R', wherein R' is a rare earth element and includes Pr and Nd; wherein, Pr ≥ 17.15%;
0.25-1.05% of Ga;
0.9-1.2% of B;
64-69% of Fe; **characterised in that**
Cu ≥ 0.35%;
Al ≤ 0.03%;
0.25-0.3% of Zr.

2. The raw material composition according to claim 1, wherein, the content of Pr is 17.15-29%, preferably 17.15%, 18.15%, 19.15%, 20.15%, 21.15%, 22.15%, 23.15%, 24.15%, 25.15%, 26.15%, 27.15%, 27.85%, or 28.85%;
and/or, the content of Nd is 1.85-14%, preferably 1.85%, 2.85%, 3.85%, 4.85%, 5.85%, 6.15%, 6.85%, 7.85%, 8.85%, 9.85%, 10.65%, 10.85%, 11.15%, 11.35%, 11.75%, 12.35%, 12.85%, 13.65%, or 13.85%;
and/or, the ratio of the mass of Nd to the total mass of R' is 0.5 or less, preferably 0.1-0.45; and/or, the R' further comprises other rare earth elements besides Pr and Nd, preferably Y; and/or, R' further comprises RH, RH is a heavy rare earth element; preferably, the type of RH includes one or more of Dy, Tb and Ho, more preferably Dy and/or Tb; the mass ratio of RH to R' is preferably <0.253, more preferably 0-0.07%; preferably, the content of RH is 1-2.5%; when RH contains Tb, the content of Tb is preferably 0.5%-2%, when RH contains Dy, the content of Dy is preferably 1% or less; when RH contains Ho, the content of Ho is preferably 0.8-2%%;
and/or, the content of Ga is 0.25-1%, preferably 0.25%, 0.27%, 0.28%, 0.29%, 0.3%, 0.31%, 0.32%, 0.33%, 0.35%, 0.36%, 0.37%, 0.38%, 0.39%, 0.4%, 0.41%, 0.43%, 0.45%, 0.47%, 0.49%, 0.5%, 0.51%, 0.53%, 0.55%, 0.57%, 0.6%, 0.7%, 0.8%, 0.85%, 0.9%, 0.95%, or 1%;
and/or, the content of B is 0.95-1.2%, preferably 0.95%, 0.96%, 0.97%, 0.98%, 0.985%, 1%, 1.1%, or 1.2%;
and/or, the content of Fe is 65-68.3%, preferably 65.015%, 65.215%, 65.315%, 65.335%, 65.55%, 65.752%, 65.87%, 65.985%, 66.015%, 66.165%, 66.185%, 66.315%, 66.395%, 66.405%, 66.415%, 66.465%, 66.475%, 66.515%, 66.537%, 66.602%, 66.605%, 66.615%, 66.62%, 66.665%, 66.695%, 66.755%, 66.785%, 66.915%, 66.915%, 66.935%, 67.005%, 67.055%, 67.065%, 67.085%, 67.125%, 67.145%, 67.185%, 67.195%, 67.215%, 67.245%, 67.31%, 67.315%, 67.325%, 67.415%, 67.42%, 67.54%, 67.57%, 67.6%, 67.705%, 67.745%, 67.765%, 67.795%, 67.815%, 68.065%, or 68.225%;
and/or, the raw material composition of neodymium-iron-boron magnet material further comprises Cu; preferably, the content of Cu is 0.35 -0.8%, preferably
0.35%, 0.4%, 0.45%, 0.48%, 0.5%, 0.55%, 0.58%, 0.7%, or 0.8%;
and/or, the raw material composition of neodymium-iron-boron magnet material further comprises Al; preferably, the content of Al is 0.01-0.03% preferably 0.02%, or 0.03%
and/or, the raw material composition of neodymium-iron-boron magnet material further comprises Zr; preferably, the content of Zr is 0.25%, 0.26%, 0.27%, 0.28%, 0.29%, or 0.3%;
and/or, the raw material composition of neodymium-iron-boron magnet material further comprises Co; preferably, the content of Co is 0.5-2%;
and/or, the raw material composition of neodymium-iron-boron magnet material further comprises Mn; preferably, the content of Mn is 0.02% or less, preferably 0.01%, 0.013%, 0.015%, or 0.018%;
and/or, the raw material composition of neodymium-iron-boron magnet material further comprise one or more of Zn, Ag, In, Sn, V, Cr, Mo, Ta, Hf and W; the content of Zn is preferably 0.1% or less, more preferably 0.01-0.08%; wherein, the content of Mo is preferably 0.1% or less, more preferably 0.01-0.08%.

3. The raw material composition according to claim 1 or 2, wherein R' further comprises RH, RH is heavy rare earth element, the content of RH is preferably 1-2.5%; the content of Cu is preferably 0.35 -0.8%; the content of Pr is preferably 17.15-29%.

4. The raw material composition according to claim 1 or 2, which comprises the following components by mass percentage: 29.5-32% of R', R' is a rare-earth element and includes Pr and Nd; wherein, Pr≥17.15%; 0.25-1.05% of Ga; Mn≤0.02%; 0.25-0.3% of Zr; 0.9-1.2% of B; 64-69% of Fe;
preferably, R' further comprises RH, RH is heavy rare earth element, the content of RH is preferably 1-2.5%; the content of Pr is preferably 17.15-29%; the content of Ga is preferably 0.8-1%.

5. A preparation method for neodymium-iron-boron magnet material, which employs the raw material composition according to any one of claims 1-4 for preparing;
preferably, the preparation method comprises the following steps: the molten liquid of the raw material composition according to any one of claims 1-4 is subjected to melting and casting, hydrogen decrepitation, forming, sintering and ageing treatment.

6. A neodymium-iron-boron magnet material, which comprises the following components by mass percentage, wherein the percentage refers to the mass percentage of the content of each component in the total mass of the raw material composition of neodymium-iron-boron magnet material:
29.5-32% of R', R' comprises Pr and Nd; wherein, Pr≥17.15%;
0.245-1.05% of Ga;
0.9-1.2% of B;
64-69% of Fe; **characterised in that**
0.35-0.9% of Cu;
≤0.03 % of Al;
0.25-0.3% of Zr.

7. The neodymium-iron-boron magnet material according to claim 6, wherein, the content of Pr is 17.15-29%, preferably 17.145%, 17.147%, 17.149%, 17.15%, 17.151%, 17.152%, 18.132%, 18.146%, 18.148%, 19.146%, 19.148%, 19.149%, 19.149%, 19.151%, 19.153%, 20.146%, 20.147%, 20.148%, 20.149%, 20.151%, 20.154%, 21.146%, 21.148%, 22.148%, 23.147%, 23.148%, 23.149%, 23.15%, 23.151%, 23.152%, 24.148%, 24.151%, 24.152%, 25.152%, 26.151%, 27.152%, 27.851%, or 28.852%;
and/or, the content of Nd is 1.85-14%, preferably 1.852%, 2.848%, 3.848%, 4.852%, 5.845%, 5.848%, 5.85%, 5.851%, 5.852%, 6.147%, 6.148%, 6.149%, 6.151%, 6.846%, 6.847%, 6.848%, 6.853%, 7.846%, 7.849%, 7.851%, 7.852%, 8.851%, 9.549%, 9.848%, 9.851%, 9.852%, 10.651%, 10.848%, 10.849%, 10.851%, 11.148%, 11.149%, 11.352%, 11.355%, 11.746%, 11.747%, 11.748%, 11.751%, 11.752%, 12.345%, 12.347%, 12.35%, 12.451%, 12.848%, 12.851%, 12.89%, 13.348%, 13.651%, 13.848%, 13.849%, or 13.856%;
and/or, the ratio of the mass of Nd to the total mass of R' is <0.5, preferably 0.06-0.45; and/or, R' further comprises other rare earth elements besides Pr and Nd, preferably Y; and/or, R' further comprises RH, RH is a heavy rare earth element, the kind of RH preferably comprises one or more of Dy, Tb and Ho, preferably Dy and/or Tb; preferably, the mass ratio of RH and R' is preferably <0.253, more preferably 0.01-0.07; the content of RH is preferably 1-2.5%; wherein, when RH comprises Tb, the content of Tb is 0.5-2.01%; wherein, when RH comprises Dy, the content of Dy is 1.05% or less, preferably 0.1-1.03%; wherein, when RH comprises Ho, the content of Ho is preferably 0.8-2%%;
and/or, the content of Ga is 0.247-1.03%, preferably 0.247%, 0.248%, 0.249%, 0.251%, 0.252%, 0.268%, 0.281%, 0.291%, 0.3%, 0.301%, 0.302%, 0.303%, 0.312%, 0.323%, 0.332%, 0.351%, 0.352%, 0.361%, 0.362%, 0.371%, 0.38%, 0.392%, 0.402%, 0.413%, 0.433%, 0.45%, 0.451%, 0.452%, 0.471%, 0.472%, 0.491%, 0.492%, 0.502%, 0.512%, 0.531%, 0.55%, 0.551%, 0.572%, 0.589%, 0.6%, 0.602%, 0.701%, 0.703%, 0.712%, 0.791%, 0.804%, 0.82%, 0.848%, 0.892%, 0.912%, 0.951%, 1.02%, or 1.03%;
and/or, the content of B is preferably 0.95-1.2%, preferably 0.949%, 0.956%, 0.969%, 0.982%, 0.983%, 0.984%, 0.985%, 0.986%, 0.987%, 0.991%, 1.02%, 1.11%, 1.18%, or 1.19%;
and/or, the content ofFe is 64.8-68.2%, preferably 64.981%, 65.157%, 65.296%, 65.308%, 65.54%, 65.729%, 65.849%, 65.9895, 66.002%, 66.15%, 66.209%, 66.296%, 66.392%, 66.393%, 66.404%, 66.445%, 66.451%, 66.458, 66.503%, 66.532%, 66.595%, 66.607%, 66.6145, 66.62%, 66.644%, 66.664%, 66.756%, 66.782%, 66.909%, 66.912%, 66.913%, 66.941%, 67.007%, 67.058%, 67.072%, 67.093%, 67.125%, 67.14%, 67.187%, 67.188%, 67.195%, 67.247%, 67.267%, 67.279%, 67.294%, 67.327%, 67.347%, 67.405%, 67.425, 67.468, 67.47%, 67.517%, 67.535%, 67.571%, 67.6%, 67.621%, 67.667%, 67.739%, 67.769%, 67.801%, 67.813%, 67.816%, 68.07%, or 68.143%;
and/or, the neodymium-iron-boron magnet material further comprises Cu; preferably, the content of Cu is 0.35-0.9%,
more preferably 0.351%, 0.352%, 0.402%, 0.405%, 0.451%, 0.452%, 0.481%, 0.5%, 0.501%, 0.502%, 0.552%, 0.581%, 0.7%, or 0.803%;
and/or, the neodymium-iron-boron magnet material further comprises Al; preferably, the content of Al is 0.01-0.03%;
and/or, the neodymium-iron-boron magnet material further comprises Zr; preferably, the content of Zr is 0.3% or less;
and/or, the neodymium-iron-boron magnet material further comprises Co; preferably, the content of Co is 0.5-2%;
and/or, the neodymium-iron-boron magnet material further comprises Mn; preferably, the content of Mn is 0.02% or less, more preferably 0.01%, 0.013%, 0.015%, 0.014%, 0.018%, or 0.02%;
and/or, the neodymium-iron-boron magnet material further comprises O; preferably, the content of O is 0.13% or less;
and/or, the neodymium-iron-boron magnet material may further comprise one or more of Zn, Ag, In, Sn, V, Cr, Mo, Ta, Hf and W; wherein, the content of Zn is preferably 0.1% or less, more preferably 0.01-0.08%; wherein, the content of Mo is preferably 0.1% or less, more preferably 0.01-0.08%.

8. A neodymium-iron-boron magnet material, wherein, in the intergranular triangle region of the neodymium-iron-boron magnet material, the ratio of the total mass of Pr and Ga to the total mass of Nd and Ga≤1.0;
at the grain boundary of the neodymium-iron-boron magnet material, the ratio of the total mass of Pr and Ga to the total mass of Nd and Ga;
preferably, the components of the neodymium-iron-boron magnet material refer to the neodymium-iron-boron magnet material according to any one of claims 6-7.

9. A use of the neodymium-iron-boron magnet material according to any one of claims 6-8 as an electronic component in a motor.

## Patentansprüche

1. Eine Rohmaterialzusammensetzung von Neodym-Eisen-Bor-Magnetmaterial, die die folgenden Komponenten in Massenprozent umfasst, wobei sich der Prozentsatz auf den Massenprozentsatz des Gehalts jeder Komponente in der Gesamtmasse der Rohmaterialzusammensetzung des Neodym-Eisen-Bor-Magnetmaterials bezieht:
29,5-32% R', wobei R' ein Seltenerdelement ist und Pr und Nd einschließt; wobei Pr ≥ 17,15%;
0,25-1,05% Ga;
0,9-1,2% B;
64-69% Fe; **dadurch gekennzeichnet, dass**
Cu ≥ 0,35%;
AI ≤ 0,03%;
0,25-0,3% Zr.

2. Rohmaterialzusammensetzung nach Anspruch 1, wobei der Gehalt an Pr 17,15-29%, vorzugsweise 17,15%, 18,15%, 19,15%, 20,15%, 21,15%, 22,15%, 23,15%, 24,15%, 25,15%, 26,15%, 27,15%, 27,85% oder 28,85% beträgt;
und/oder der Gehalt an Nd 1,85-14%, vorzugsweise 1,85%, 2,85%, 3,85%, 4,85%, 5,85%, 6,15%, 6,85%, 7,85%, 8,85%, 9,85%, 10,65%, 10,85%, 11,15%, 11,35%, 11,75%, 12,35%, 12,85%, 13,65% oder 13,85% beträgt;
und/oder das Verhältnis der Masse von Nd zur Gesamtmasse von R' 0,5 oder weniger, vorzugsweise 0,1-0,45, beträgt;
und/oder R' ferner andere Seltenerdelemente außer Pr und Nd, vorzugsweise Y, umfasst; und/oder R' ferner RH umfasst, wobei RH ein schweres Seltenerdelement ist; vorzugsweise schließt der Typ von RH eines oder mehrere von Dy, Tb und Ho, vorzugsweise Dy und/oder Tb, ein; das Massenverhältnis von RH zu R' ist vorzugsweise <0,253, mehr bevorzugt 0-0,07%; vorzugsweise beträgt der Gehalt an RH 1-2,5%; wenn RH Tb enthält, beträgt der Gehalt an Tb vorzugsweise 0,5%-2%, wenn RH Dy enthält, beträgt der Gehalt an Dy vorzugsweise 1% oder weniger; wenn RH Ho enthält, beträgt der Gehalt an Ho vorzugsweise 0,8-2%;
und/oder der Gehalt an Ga 0,25-1%, vorzugsweise 0,25%, 0,27%, 0,28%, 0,29%, 0,3%, 0,31%, 0,32%, 0,33%, 0,35%, 0,36%, 0,37%, 0,38%, 0,39%, 0,4%, 0,41%, 0,43%, 0,45%, 0,47%, 0,49%, 0,5%, 0,51%, 0,53%, 0,55%, 0,57%, 0,6%, 0,7%, 0,8%, 0,85%, 0,9%, 0,95%, oder 1% beträgt;
und/oder der Gehalt an B 0,95-1,2%, vorzugsweise 0,95%, 0,96%, 0,97%, 0,98%, 0,985%, 1%, 1,1% oder 1,2% beträgt;
und/oder der Gehalt an Fe 65-68,3%, vorzugsweise 65,015%, 65,215%, 65,315%, 65,335%, 65,55%, 65,752%, 65,87%, 65,985%, 66,015%, 66,165%, 66,185%, 66,315%, 66,395%, 66,405%, 66,415%, 66,465%, 66,475%, 66,515%, 66,537%, 66,602%, 66,605%, 66,615%, 66,62%, 66,665%, 66,695%, 66,755%, 66,785%, 66,915%, 66,915%, 66,935%, 67,005%, 67,055%, 67,065%, 67,085%, 67,125%, 67,145%, 67,185%, 67,195%, 67,215%, 67,245%, 67,31%, 67,315%, 67,325%, 67,415%, 67,42%, 67,54%, 67,57%, 67,6%, 67,705%, 67,745%, 67,765%, 67,795%, 67,815%, 68,065%, oder 68,225% beträgt;
und/oder die Rohmaterialzusammensetzung des Neodym-Eisen-Bor-Magnetmaterials ferner Cu umfasst; vorzugsweise beträgt der Gehalt an Cu 0,35-0,8%, vorzugsweise 0,35%, 0,4%, 0,45%, 0,48%, 0,5%, 0,55%, 0,58%, 0,7% oder 0,8%;
und/oder die Rohmaterialzusammensetzung des Neodym-Eisen-Bor-Magnetmaterials ferner Al umfasst; vorzugsweise beträgt der Gehalt an Al 0,01-0,03%, vorzugsweise 0,02% oder 0,03%;
und/oder die Rohmaterialzusammensetzung des Neodym-Eisen-Bor-Magnetmaterials ferner Zr umfasst; vorzugsweise beträgt der Gehalt an Zr 0,25%, 0,26%, 0,27%, 0,28%, 0,29% oder 0,3%;
und/oder die Rohmaterialzusammensetzung des Neodym-Eisen-Bor-Magnetmaterials ferner Co umfasst; vorzugsweise beträgt der Gehalt an Co 0,5-2%;
und/oder die Rohmaterialzusammensetzung des Neodym-Eisen-Bor-Magnetmaterials ferner Mn umfasst; vorzugsweise beträgt der Gehalt an Mn 0,02% oder weniger, vorzugsweise 0,01%, 0,013%, 0,015% oder 0,018%;
und/oder die Rohmaterialzusammensetzung des Neodym-Eisen-Bor-Magnetmaterials ferner eines oder mehrere von Zn, Ag, In, Sn, V, Cr, Mo, Ta, Hf und W umfasst; der Gehalt an Zn beträgt vorzugsweise 0,1% oder weniger, mehr bevorzugt 0,01-0,08%; wobei der Gehalt an Mo vorzugsweise 0,1% oder weniger, mehr bevorzugt 0,01-0,08% beträgt.

3. Rohmaterialzusammensetzung nach Anspruch 1 oder 2, wobei R' ferner RH umfasst, RH ist ein schweres Seltenerdelement, der Gehalt an RH beträgt vorzugsweise 1-2,5%; der Gehalt an Cu beträgt vorzugsweise 0,35-0,8%; der Gehalt an Pr beträgt vorzugsweise 17,15-29%.

4. Rohmaterialzusammensetzung nach Anspruch 1 oder 2, die die folgenden Komponenten in Massenprozent umfasst: 29,5-32% R', R' ist ein Seltenerdelement und schließt Pr und Nd ein; wobei Pr≥17,15%; 0,25-1,05% Ga; Mn≤0,02%; 0,25-0,3% Zr; 0,9-1,2% B; 64-69% Fe; vorzugsweise umfasst R' ferner RH, RH ist ein schweres Seltenerdelement, der Gehalt an RH beträgt vorzugsweise 1-2,5%; der Gehalt an Pr beträgt vorzugsweise 17,15-29%; der Gehalt an Ga beträgt vorzugsweise 0,8-1%.

5. Ein Herstellungsverfahren für Neodym-Eisen-Bor-Magnetmaterial, bei dem die Rohstoffzusammensetzung nach einem der Ansprüche 1-4 zur Herstellung verwendet wird; vorzugsweise umfasst das Herstellungsverfahren die folgenden Schritte: Die geschmolzene Flüssigkeit der Rohstoffzusammensetzung nach einem der Ansprüche 1-4 wird einer Schmelz- und Gießbehandlung, einer Wasserstoffdekrepitation, einer Formgebung, einer Sinterung und einer Alterungsbehandlung unterzogen.

6. Ein Neodym-Eisen-Bor-Magnetmaterial, das die folgenden Komponenten in Massenprozent umfasst, wobei sich der Prozentsatz auf den Massenprozentsatz des Gehalts jeder Komponente an der Gesamtmasse der Rohmaterialzusammensetzung des Neodym-Eisen-Bor-Magnetmaterials bezieht:
29,5-32% von R', R' umfasst Pr und Nd; wobei Pr≥17,15%;
0,245-1,05% Ga;
0,9-1,2% B;
64-69% Fe; **dadurch gekennzeichnet, dass**
0,35-0,9% Cu;
≤0,03% Al;
0,25-0,3% Zr.

7. Neodym-Eisen-Bor-Magnetmaterial nach Anspruch 6, wobei der Gehalt an Pr 17,15-29%, vorzugsweise 17,145%, 17,147%, 17,149%, 17,15%, 17,151%, 17,152%, 18,132%, 18,146%, 18,148%, 19,146%, 19,148%, 19,149%, 19,149%, 19,151%, 19,153%, 20,146%, 20,147%, 20,148%, 20,149%, 20,151%, 20,154%, 21,146%, 21,148%, 22,148%, 23,147%, 23,148%, 23,149%, 23,15%, 23,151%, 23,152%, 24,148%, 24,151%, 24,152%, 25,152%, 26,151%, 27,152%, 27,851%, oder 28,852% beträgt;
und/oder der Gehalt an Nd 1,85-14%, vorzugsweise 1,852%, 2,848%, 3,848%, 4,852%, 5,845%, 5,848%, 5,85%, 5,851%, 5,852%, 6,147%, 6,148%, 6,149%, 6,151%, 6,846%, 6,847%, 6,848%, 6,853%, 7,846%, 7,849%, 7,851%, 7,852%, 8,851%, 9,549%, 9,848%, 9,851%, 9,852%, 10,651%, 10,848%, 10,849%, 10,851%, 11,148%, 11,149%, 11,352%, 11,355%, 11,746%, 11,747%, 11,748%, 11,751%, 11,752%, 12,345%, 12,347%, 12,35%, 12,451%, 12,848%, 12,851%, 12,89%, 13,348%, 13,651%, 13,848%, 13,849% oder 13,856% beträgt;
und/oder das Verhältnis der Masse von Nd zur Gesamtmasse von R' <0,5, vorzugsweise 0,06-0,45 ist;
und/oder R' ferner andere Seltenerdelemente neben Pr und Nd, vorzugsweise Y, umfasst; und/oder R' ferner RH umfasst, RH ist ein schweres Seltenerdelement, die Art von RH umfasst vorzugsweise eines oder mehrere von Dy, Tb und Ho, vorzugsweise Dy und/oder Tb; das Massenverhältnis von RH und R' beträgt vorzugsweise <0,253, mehr bevorzugt 0,01-0,07; der Gehalt an RH beträgt vorzugsweise 1-2,5%; wobei, wenn RH Tb umfasst, der Gehalt an Tb 0,5-2,01% beträgt; wobei, wenn RH Dy umfasst, der Gehalt an Dy 1,05% oder weniger, vorzugsweise 0,1-1,03% beträgt; wobei, wenn RH Ho umfasst, der Gehalt an Ho vorzugsweise 0,8-2% beträgt;
und/oder der Gehalt an Ga 0,247-1,03%, vorzugsweise 0,247%, 0,248%, 0,249%, 0,251%, 0,252%, 0,268%, 0,281%, 0,291%, 0,3%, 0,301%, 0,302%, 0,303%, 0,312%, 0,323%, 0,332%, 0,351%, 0,352%, 0,361%, 0,362%, 0,371%, 0,38%, 0,392%, 0,402%, 0,413%, 0,433%, 0,45%, 0,451%, 0,452%, 0,471%, 0,472%, 0,491%, 0,492%, 0,502%, 0,512%, 0,531%, 0,55%, 0,551%, 0,572%, 0,589%, 0,6%, 0,602%, 0,701%, 0,703%, 0,712%, 0,791%, 0,804%, 0,82%, 0,848%, 0,892%, 0,912%, 0,951%, 1,02%, oder 1,03% beträgt; und/oder der Gehalt an B vorzugsweise 0,95-1,2%, vorzugsweise 0,949%, 0,956%, 0,969%, 0,982%, 0,983%, 0,984%, 0,985%, 0,986%, 0,987%, 0,991%, 1,02%, 1,11%, 1,18% oder 1,19% beträgt;
und/oder der Gehalt an Fe 64,8-68,2%, vorzugsweise 64,981%, 65,157%, 65,296%, 65,308%, 65,54%, 65,729%, 65,849%, 65,9895, 66,002%, 66,15%, 66,209%, 66,296%, 66,392%, 66,393%, 66,404%, 66,445%, 66,451%, 66,458, 66,503%, 66,532%, 66,595%, 66,607%, 66,6145, 66,62%, 66,644%, 66,664%, 66,756%, 66,782%, 66,909%, 66, 912%, 66,913%, 66,941%, 67,007%, 67,058%, 67,072%, 67,093%, 67,125%, 67,14%, 67,187%, 67,188%, 67,195%, 67,247%, 67,267%, 67,279%, 67,294%, 67,327%, 67,347%, 67,405%, 67,425, 67,468, 67,47%, 67,517%, 67,535%, 67,571%, 67,6%, 67,621%, 67,667%, 67,739%, 67,769%, 67,801%, 67,813%, 67,816%, 68,07%, oder 68,143% beträgt;
und/oder das Neodym-Eisen-Bor-Magnetmaterial ferner Cu umfasst; vorzugsweise beträgt der Gehalt an Cu 0,35-0,9%, mehr bevorzugt 0,351%, 0,352%, 0,402%, 0,405%, 0,451%, 0,452%, 0,481%, 0,5%, 0,501%, 0,502%, 0,552%, 0,581%, 0,7% oder 0,803%;
und/oder das Neodym-Eisen-Bor-Magnetmaterial ferner Al umfasst; vorzugsweise beträgt der Gehalt an Al 0,01-0,03 %;
und/oder das Neodym-Eisen-Bor-Magnetmaterial ferner Zr umfasst; vorzugsweise beträgt der Gehalt an Zr 0,3 % oder weniger;
und/oder das Neodym-Eisen-Bor-Magnetmaterial ferner Co umfasst; vorzugsweise beträgt der Gehalt an Co 0,5-2%;
und/oder das Neodym-Eisen-Bor-Magnetmaterial ferner Mn umfasst; vorzugsweise beträgt der Gehalt an Mn 0,02% oder weniger, mehr bevorzugt 0,01%, 0,013%, 0,015%, 0,014%, 0,018% oder 0,02%;
und/oder das Neodym-Eisen-Bor-Magnetmaterial ferner O enthält; vorzugsweise beträgt der Gehalt an O 0,13% oder weniger;
und/oder das Neodym-Eisen-Bor-Magnetmaterial ferner eines oder mehrere der Elemente Zn, Ag, In, Sn, V, Cr, Mo, Ta, Hf und W umfassen kann; wobei der Gehalt an Zn vorzugsweise 0,1% oder weniger, mehr bevorzugt 0,01-0,08%, beträgt; wobei der Gehalt an Mo vorzugsweise 0,1% oder weniger, mehr bevorzugt 0,01-0,08%, beträgt.

8. Ein Neodym-Eisen-Bor-Magnetmaterial, wobei in dem intergranularen Dreiecksbereich des Neodym-Eisen-Bor-Magnetmaterials das Verhältnis der Gesamtmasse von Pr und Ga zur Gesamtmasse von Nd und Ga ≤1,0 ist;
an der Korngrenze des Neodym-Eisen-Bor-Magnetmaterials das Verhältnis der Gesamtmasse von Pr und Ga zu der Gesamtmasse von Nd und Ga;
vorzugsweise beziehen sich die Komponenten des Neodym-Eisen-Bor-Magnetmaterials auf das Neodym-Eisen-Bor-Magnetmaterial nach einem der Ansprüche 6-7.

9. Verwendung des Neodym-Eisen-Bor-Magnetmaterials nach einem der Ansprüche 6-8 als elektronisches Bauteil in einem Motor.

## Revendications

1. Composition de matière première de matériau magnétique néodyme-fer-bore, qui comprend les composants suivants en pourcentage en masse, dans laquelle le pourcentage se réfère au pourcentage en masse de la teneur de chaque composant dans la masse totale de la composition de matière première de matériau magnétique néodyme-fer-bore :
29,5-32 % de R', dans laquelle R' est un élément de terre rare et comprend Pr et Nd ; dans laquelle Pr ≥ 17,15 % ;
de 0,25 à 1,05 % de Ga ;
de 0,9 à 1,2 % de B ;
de 64 à 69 % de Fe ; **caractérisée en ce que**
Cu ≥ 0,35 %
Al ≤ 0,03 %
de 0,25 à 0,3 % de Zr.

2. Composition de matière première selon la revendication 1, dans laquelle la teneur en Pr est de 17,15 à 29 %, de préférence de 17,15 %, 18,15 %, 19,15 %, 20,15 %, 21,15 %, 22,15 %, 23,15 %, 24,15 %, 25,15 %, 26,15 %, 27,15 %, 27,85 % ou 28,85 % ;
et/ou, la teneur en Nd est de 1,85 à 14 %, de préférence de 1,85 %, 2,85 %, 3,85 %, 4,85 %, 5,85 %, 6,15 %, 6,85 %, 7,85 %, 8,85 %, 9,85 %, 10,65 %, 10,85 %, 11,15 %, 11,35 %, 11,75 %, 12,35 %, 12,85 %, 13,65 % ou 13,85 % ;
et/ou, le rapport de la masse de Nd à la masse totale de R' est de 0,5 ou moins, de préférence de 0,1 à 0,45 ;
et/ou, le R' comprend en outre d'autres éléments de terres rares en plus de Pr et Nd, de préférence Y ;
et/ou, R' comprend en outre RH, RH est un élément de terre rare lourd ; de préférence, le type de RH comprend un ou plusieurs éléments parmi Dy, Tb et Ho, plus préférablement Dy et/ou Tb ; le rapport massique de RH à R' est de préférence <0,253, plus préférablement de 0 à 0,07 % ; de préférence, la teneur en RH est de 1 à 2,5 % ; lorsque RH contient Tb, la teneur en Tb est de préférence de 0,5 % à 2 %, lorsque RH contient Dy, la teneur en Dy est de préférence de 1 % ou moins ; lorsque RH contient Ho, la teneur en Ho est de préférence de 0,8 à 2 %% ;
et/ou, la teneur en Ga est de 0,25 à 1 %, de préférence de 0,25 %, 0,27 %, 0,28 %, 0,29 %, 0,3 %, 0,31 %, 0,32 %, 0,33 %, 0,35 %, 0,36 %, 0,37 %, 0,38 %, 0,39 %, 0,4 %, 0,41 %, 0,43 %, 0,45 %, 0,47 %, 0,49 %, 0,5 %, 0,51 %, 0,53 %, 0,55 %, 0,57 %, 0,6 %, 0,7 %, 0,8 %, 0,85 %, 0,9 %, 0,95 % ou 1 % ;
et/ou, la teneur en B est de 0,95 à 1,2 %, de préférence de 0,95 %, 0,96 %, 0,97 %, 0,98 %, 0,985 %, 1 %, 1,1 % ou 1,2 % ;
et/ou, la teneur en Fe est de 65 à 68,3 %, de préférence de 65,015 %, 65,215 %, 65,315 %, 65,335 %, 65,55 %, 65,752 %, 65,87 %, 65,985 %, 66,015 %, 66,165 %, 66,185 %, 66,315 %, 66,395 %, 66,405 %, 66,415 %, 66,465 %, 66,475 %, 66,515 %, 66,537 %, 66,602 %, 66,605 %, 66,615 %, 66,62 %, 66,665 %, 66,695 %, 66,755 %, 66,785 %, 66,915 %, 66,915 %, 66,935 %, 67,005 %, 67,055 %, 67,065 %, 67,085 %, 67,125 %, 67,145 %, 67,185 %, 67,195 %, 67,215 %, 67,245 %, 67,31 %, 67,315 %, 67,325 %, 67,415 %, 67,42 %, 67,54 %, 67,57 %, 67,6 %, 67,705 %, 67,745 %, 67,765 %, 67,795 %, 67,815 %, 68,065 %, ou 68,225 % ;
et/ou, la composition de matière première du matériau magnétique néodyme-fer-bore comprend en outre du Cu ; de préférence, la teneur en Cu est de 0,35 à 0,8 %, de préférence de 0,35 %, 0,4 %, 0,45 %, 0,48 %, 0,5 %, 0,55 %, 0,58 %, 0,7 % ou 0,8 % ; et/ou, la composition de matière première du matériau magnétique néodyme-fer-bore comprend en outre Al ; de préférence, la teneur en Al est de 0,01 à 0,03 %, de préférence de 0,02 %, ou 0,03 % ;
et/ou, la composition de matière première du matériau magnétique néodyme-fer-bore comprend en outre du Zr ; de préférence, la teneur en Zr est de 0,25 %, 0,26 %, 0,27 %, 0,28 %, 0,29 % ou 0,3 % ;
et/ou, la composition de matière première du matériau magnétique néodyme-fer-bore comprend en outre du Co ; de préférence, la teneur en Co est de 0,5 à 2% ;
et/ou, la composition de matière première du matériau magnétique néodyme-fer-bore comprend en outre du Mn ; de préférence, la teneur en Mn est de 0,02 % ou moins, de préférence de 0,01 %, 0,013 %, 0,015 % ou 0,018 % ;
et/ou, la composition de matière première du matériau magnétique néodyme-fer-bore comprend en outre un ou plusieurs éléments parmi Zn, Ag, In, Sn, V, Cr, Mo, Ta, Hf et W ; la teneur en Zn est de préférence de 0,1 % ou moins, plus préférablement de 0,01 à 0,08 %; dans laquelle, la teneur en Mo est de préférence de 0,1 % ou moins, plus préférablement de 0,01 à 0,08 %.

3. Composition de matière première selon la revendication 1 ou 2, dans laquelle R' comprend en outre RH, RH est un élément de terre rare lourde, la teneur en RH est de préférence de 1 à 2,5 % ; la teneur en Cu est de préférence de 0,35 à 0,8 % ; la teneur en Pr est de préférence de 17,15 à 29 %.

4. Composition de matière première selon la revendication 1 ou 2, qui comprend les composants suivants en pourcentage en masse : 29,5-32 % de R', R' est un élément de terre rare et comprend Pr et Nd ; dans laquelle Pr≥17,15 % ; de 0,25 à 1,05 % de Ga ; Mn≤0,02 % ; de 0,25 à 0,3 % de Zr ; de 0,9 à 1,2 % de B ; de 64 à 69 % de Fe ;
de préférence, R' comprend en outre RH, RH est un élément de terre rare lourde, la teneur en RH est de préférence de 1 à 2,5 % ; la teneur en Pr est de préférence de 17,15 à 29 % ; la teneur en Ga est de préférence de 0,8 à 1 %.

5. Procédé de préparation d'un matériau magnétique néodyme-fer-bore, qui utilise la composition de matière première selon l'une quelconque des revendications 1 à 4 pour la préparation ;
de préférence, le procédé de préparation comprend les étapes suivantes : le liquide fondu de la composition de matière première selon l'une quelconque des revendications 1 à 4 est soumis à un traitement de fusion et de coulée, de décrépitation d'hydrogène, de formage, de frittage et de vieillissement.

6. Matériau magnétique néodyme-fer-bore, qui comprend les composants suivants en pourcentage en masse, dans lequel le pourcentage se réfère au pourcentage en masse de la teneur de chaque composant dans la masse totale de la composition de matière première du matériau magnétique néodyme-fer-bore :
de 29,5 à 32 % de R', R' comprend Pr et Nd ; dans lequel Pr≥17,15 % ;
de 0,245 à 1,05 % de Ga ;
de 0,9 à 1,2 % de B ;
de 64 à 69 % de Fe ; **caractérisé en ce que**
de 0,35 à 0,9 % de Cu ;
≤0,03 % d'Al ;
de 0,25 à 0,3 % de Zr.

7. Matériau magnétique néodyme-fer-bore selon la revendication 6, dans lequel la teneur en Pr est de 17,15 à 29 %, de préférence de 17,145 %, 17,147 %, 17,149 %, 17,15 %, 17,151 %, 17,152 %, 18,132 %, 18,146 %, 18,148 %, 19,146 %, 19,148 %, 19,149 %, 19,149%, 19,151 %, 19,153 %, 20,146 %, 20,147 %, 20,148 %, 20,149 %, 20,151 %, 20,154 %, 21,146 %, 21,148 %, 22,148 %, 23,147 %, 23,148 %, 23,149 %, 23,15 %, 23,151 %, 23,152 %, 24,148 %, 24,151 %, 24,152 %, 25,152 %, 26,151 %, 27,152 %, 27,851 % ou 28,852 % ;
et/ou, la teneur en Nd est de 1,85 à 14 %, de préférence 1,852 %, 2,848 %, 3,848 %, 4,852 %, 5,845 %, 5,848 %, 5,85 %, 5,851 %, 5,852 %, 6,147 %, 6,148 %, 6,149 %, 6,151 %, 6,846 %, 6,847 %, 6,848 %, 6,853 %, 7,846 %, 7,849 %, 7,851 %, 7,852 %, 8,851 %, 9,549 %, 9,848 %, 9,851 %, 9,852 %, 10,651 %, 10,848 %, 10,849 %, 10,851 %, 11,148 %, 11,149 %, 11,352 %, 11,355 %, 11,746 %, 11,747 %, 11,748 %, 11,751 %, 11,752 %, 12,345 %, 12,347 %, 12,35 %, 12,451 %, 12,848 %, 12,851 %, 12,89 %, 13,348 %, 13,651 %, 13,848 %, 13,849 %, ou 13,856 % ;
et/ou, le rapport de la masse de Nd à la masse totale de R' est <0,5, de préférence de 0,06 à 0,45 ;
et/ou, R' comprend en outre d'autres éléments de terres rares en plus de Pr et Nd, de préférence Y ;
et/ou, R' comprend en outre RH, RH est un élément de terre rare lourd, le type de RH comprend de préférence un ou plusieurs éléments parmi Dy, Tb et Ho, de préférence Dy et/ou Tb ; de préférence, le rapport massique de RH et R' est de préférence <0,253, plus préférablement de 0,01 à 0,07 ; la teneur en RH est de préférence de 1 à 2,5 % ; dans lequel, lorsque RH comprend Tb, la teneur en Tb est de 0,5 à 2,01 % ; dans lequel, lorsque RH comprend Dy, la teneur en Dy est de 1,05 % ou moins, de préférence de 0,1 à 1,03 % ; dans lequel, lorsque RH comprend Ho, la teneur en Ho est de préférence de 0,8-2 %% ; et/ou, la teneur en Ga est de 0,247 à 1,03 %, de préférence de 0,247 %, 0,248 %, 0,249 %, 0,251 %, 0,252 %, 0,268 %, 0,281 %, 0,291 %, 0,3 %, 0,301 %, 0,302 %, 0,303 %, 0,312 %, 0,323 %, 0,332 %, 0,351 %, 0,352 %, 0,361 %, 0,362 %, 0,371 %, 0,38 %, 0,392 %, 0,402 %, 0,413 %, 0,433 %, 0,45 %, 0,451 %, 0,452 %, 0,471 %, 0,472 %, 0,491 %, 0,492 %, 0,502 %, 0,512 %, 0,531 %, 0,55 %, 0,551 %, 0,572 %, 0,589 %, 0,6 %, 0,602 %, 0,701 %, 0,703 %, 0,712 %, 0,791 %, 0,804 %, 0,82 %, 0,848 %, 0,892 %, 0,912 %, 0,951 %, 1,02 %, ou 1,03 % ;
et/ou, la teneur en B est de préférence de 0,95 à 1,2 %, de préférence de 0,949 %, 0,956 %, 0,969 %, 0,982 %, 0,983 %, 0,984 %, 0,985 %, 0,986 %, 0,987 %, 0,991 %, 1,02 %, 1,11 %, 1,18 % ou 1,19 % ;
et/ou, la teneur en Fe est de 64,8 à 68,2 %, de préférence de 64,981 %, 65,157 %, 65,296 %, 65,308 %, 65,54 %, 65,729 %, 65,849 %, 65,9895, 66,002 %, 66,15 %, 66,209 %, 66,296 %, 66,392 %, 66,393 %, 66,404 %, 66,445 %, 66,451 %, 66,458, 66,503 %, 66,532 %, 66,595 %, 66,607 %, 66,6145, 66,62 %, 66,644 %, 66,664 %, 66,756 %, 66,782 %, 66,909 %, 66,912 %, 66,913 %, 66,941 %, 67,007 %, 67,058 %, 67,072 %, 67,093 %, 67,125 %, 67,14 %, 67,187 %, 67,188 %, 67,195 %, 67,247 %, 67,267 %, 67,279 %, 67,294 %, 67,327 %, 67,347 %, 67,405 %, 67,425, 67,468, 67,47 %, 67,517 %, 67,535 %, 67,571 %, 67,6 %, 67,621 %, 67,667 %, 67,739 %, 67,769 %, 67,801 %, 67,813 %, 67,816 %, 68,07 %, ou 68,143 % ;
et/ou, le matériau magnétique néodyme-fer-bore comprend en outre du Cu ; de préférence, la teneur en Cu est de 0,35 à 0,9 %, plus préférablement de 0,351 %, 0,352 %, 0,402 %, 0,405 %, 0,451 %, 0,452 %, 0,481 %, 0,5 %, 0,501 %, 0,502 %, 0,552 %, 0,581 %, 0,7 % ou 0,803 % ;
et/ou, le matériau magnétique néodyme-fer-bore comprend en outre Al ; de préférence, la teneur en Al est de 0,01 à 0,03 % ;
et/ou, le matériau magnétique néodyme-fer-bore comprend en outre du Zr ; de préférence, la teneur en Zr est de 0,3 % ou moins ;
et/ou, le matériau magnétique néodyme-fer-bore comprend en outre du Co ; de préférence, la teneur en Co est de 0,5-2 % ;
et/ou, le matériau magnétique néodyme-fer-bore comprend en outre du Mn ; de préférence, la teneur en Mn est de 0,02 % ou moins, plus préférablement de 0,01 %, 0,013 %, 0,015 %, 0,014 %, 0,018 % ou 0,02 % ;
et/ou, le matériau magnétique néodyme-fer-bore comprend en outre O ; de préférence, la teneur en O est de 0,13 % ou moins ;
et/ou, le matériau magnétique néodyme-fer-bore peut en outre comprendre un ou plusieurs éléments parmi Zn, Ag, In, Sn, V, Cr, Mo, Ta, Hf et W ; dans lequel, la teneur en Zn est de préférence de 0,1 % ou moins, plus préférablement de 0,01 à 0,08 % ; dans lequel, la teneur en Mo est de préférence de 0,1 % ou moins, plus préférablement de 0,01 à 0,08 %.

8. Matériau magnétique néodyme-fer-bore, dans lequel, dans la région du triangle intergranulaire du matériau magnétique néodyme-fer-bore, le rapport de la masse totale de Pr et Ga à la masse totale de Nd et Ga≤1,0 ;
à la limite de grain du matériau magnétique néodyme-fer-bore, le rapport de la masse totale de Pr et Ga à la masse totale de Nd et Ga ;
de préférence, les composants du matériau magnétique néodyme-fer-bore se réfèrent au matériau magnétique néodyme-fer-bore selon l'une quelconque des revendications 6 à 7.

9. Utilisation du matériau magnétique néodyme-fer-bore selon l'une quelconque des revendications 6 à 8 en tant que composant électronique dans un moteur.
